

Jan. 31, 1956

E. O. FORSTER

2,733,209

MAGNESIUM-LITHIUM-SODIUM GREASE COMPOSITION

Filed Dec. 13, 1952

FIGURE-1



Eric O. Forster Inventor

By *Lawn M. Thomas* Attorney

1

2,733,209

## MAGNESIUM-LITHIUM-SODIUM GREASE COMPOSITION

Eric O. Forster, Hillside, N. J., assignor to Esso Research and Engineering Company, a corporation of Delaware

Application December 13, 1952, Serial No. 325,837

5 Claims. (Cl. 252—40)

This invention relates to lubricating grease compositions and particularly to improved magnesium grease compositions which have excellent heat stability properties. More particularly the invention relates to a heat stable magnesium grease composition containing the magnesium, lithium, and sodium soaps of fatty acids.

Magnesium base greases are well known in the art of lubricating grease manufacture. They are characterized by excellent appearance and by their resistance to shear breakdown. It has been found, however, that magnesium base greases are somewhat lacking in stability properties at sustained high temperatures. When utilized for the lubrication of moving metal parts at high temperatures for long periods of time these otherwise excellent lubricants have been found to harden to an undesirable extent and to allow oil to separate. This combination of a tendency to harden and to separate oil is an undesirable one and many attempts have been made to modify magnesium base greases to remove it.

One line of research in this direction has been the incorporation of metallic soaps, such as sodium soaps, potassium soaps and the like. This has not been satisfactory in that while the addition of these soaps decreases the tendency of the magnesium grease to harden, it increases the amount of oil separation under conditions of sustained high temperatures.

It has now been found and forms the object of this invention that the incorporation of minor amounts of both a sodium soap and a lithium soap in a magnesium base grease results in a composition that has the excellent structure stability and appearance of the magnesium greases of the prior art and in addition removes their tendency to become hard and to separate oil under conditions of sustained high temperature. This combination of properties makes these new grease compositions extremely useful in lubrication applications such as in the sealed bearings of electric motors, railroad anti-friction bearings, and automotive bearings. The compositions of this invention demonstrate a combination of desirable properties which are surprising and unexpected when compared with the results of incorporating either sodium or lithium soaps alone in a magnesium base grease.

The greases of this invention are prepared by thickening to a grease consistency a lubricating oil base stock with a mixture of the magnesium, lithium and sodium soaps of any of the well known fatty acids familiar to lubricating grease makers. The greases of invention are prepared by the methods of manufacture familiar to the art and no special problems arise in their preparation. Care must be taken only to prepare the most insoluble soap first, followed by the lesser soluble and most soluble soaps in that order.

Briefly, the preparation involves the thorough admixture of the fatty acids used in a portion of the mineral oil base and the application of heat until a homogeneous mixture is obtained. A slurry or solution of the metallic base usually in the form of hydroxide is then added and

2

the mixture heated to dehydration temperatures. On completion of dehydration the total mixture is heated to about 300° F., the balance of the mineral oil added and the final product cooled without stirring.

5 The lubricating oil chosen as the base for the grease compositions of this invention may be any of the mineral oil distillates known to the art. It should be remembered that the oil chosen for the grease base should be selected from those which would perform the lubrication if an oil alone could be used. Paraffinic or naphthenic distillates having viscosities within the range of from 35 to 1000 SUS, preferably 40 to 250 SUS at 210° F. may be utilized as the base for these improved magnesium greases. The lubricating oil constituent of these compositions may 15 also be selected from a great number of the synthetic lubricants which are rapidly becoming important in the lubricating art. Exemplary of these synthetic lubes are the long chain esters, esters of dibasic acids such as sebacic and adipic acid esters, polymerized hydrocarbons such as polyolefins, polymerized cracked wax, etc., alkylated aromatics, polyglycols, polyglycol ethers, polyglycol esters, polyglycol ether esters, formals of hydroxyl-containing compounds, etc.

25 As was stated above there is nothing critical in the fatty acid used to form the thickeners for these new grease compositions. The acid chosen may be selected from a great number of commercially available fatty acids which include stearic acid, oleic acid, hydroxy stearic acid, hydrogenated fish oil acid, beef fat, tallow, the unsaturated 30 glycerides of various fatty acids or mixtures of the above in any proportion. The acids may be used with or without plasticizers such as the polyethylene glycols and the like.

35 The thickening agent of the greases of invention consists of a mixture of the magnesium, lithium and sodium soaps of the above mentioned acids. The ratio of the three soaps used will vary from about 5 to 1 to 1 mols of magnesium, lithium and sodium soaps, respectively, to about 1 to 5 to 5 mols. The preferred compositions 40 of the invention will contain about one-half molar proportion of lithium and sodium soaps to each mol of magnesium soap.

45 The amount of the total soap mixture that is utilized in preparing the greases will depend upon the consistency desired in the final product. Ordinarily from about 5.0% by weight to about 30.0% will be used with from 10.0% to 25.0% by weight of the total mixture being especially preferred.

50 The instant invention will be more clearly explained by reference to the following representative examples.

## EXAMPLE I

## Formulation

|    | Ingredients:                             | Weight percent |
|----|------------------------------------------|----------------|
| 55 | Hydrogenated fish oil acids              | 22.00          |
|    | Magnesium hydroxide                      | 4.15           |
|    | Lithium hydroxide                        | 0.70           |
|    | Sodium hydroxide                         | 1.00           |
| 60 | Mineral lubricating oil (70 SUS/210° F.) | 72.15          |

## Preparation

65 The total charge of the hydrogenated fish oil acids and one-third of the mineral oil were mixed and heated until a homogeneous solution was obtained. An oil slurry of the magnesium hydroxide was then added and the magnesium soap allowed to form. Thereupon an aqueous solution of lithium hydroxide was added and the lithium soap formed. Upon completion of this reaction an aqueous solution of the sodium hydroxide was added and the sodium soap was prepared. The total mixture was then

## 3

heated to 240° F. and dehydrated. After all the water was driven off the temperature was raised to 300° F. and the remainder of the mineral oil was added gradually with stirring. Upon completion of the addition of the mineral oil the product was cooled without further stirring.

## EXAMPLE II

## Formulation

| Ingredients:                                | Weight per cent |
|---------------------------------------------|-----------------|
| Hydrogenated fish oil acids                 | 20.00           |
| Magnesium hydroxide                         | 4.15            |
| Lithium hydroxide                           | 1.40            |
| Mineral lubricating oil (70 SUS at 210° F.) | 74.45           |

## 4

## Preparation

This composition was prepared as in Example I except that no magnesium or lithium soaps were formed.

The grease compositions prepared as described above were tested for high temperature stability by placing samples in an oven heated at 250° F. The samples were subjected to this high temperature for 500 hours. At stated intervals during the test period samples were subjected to the micro-penetration test and after 500 hours micro-penetrations were again taken. The samples were also then examined for oil separation and appearance. Results of these tests showing the outstanding advantage of the compositions of invention are set out in Table I below.

TABLE I.—HIGH TEMPERATURE GREASE STABILITY  
500 HRS. OVEN TEST AT 250° F.

| Ex. No. | Soap Base | Percent<br>Acids | Micro-Pen. in<br>mm./10 at 77° F. |       | Dropping<br>Point, ° F. |       | Oil Sep. | Appearance<br>at the End<br>of 500 Hrs. |
|---------|-----------|------------------|-----------------------------------|-------|-------------------------|-------|----------|-----------------------------------------|
|         |           |                  | Initial                           | Final | Initial                 | Final |          |                                         |
| I       | Mg-Na-Li  | 22               | 29                                | 30    | 260                     | 255   | None     | As original.                            |
| IV      | Mg        | 20               | 43                                | 23    | 194                     | 190   | Consid.  | Buttery.                                |
| VI      | Na        | 14               | 105                               | 350   | 341                     | 330   | Slight   | Soupy.                                  |
| V       | Li        | 10               | 60                                | 320   | 234                     | 230   | do       | Soft.                                   |
| II      | Mg-Li     | 20               | 37                                | 44    | 312                     | 321   | do       | Brittle.                                |
| III     | Mg-Na     | 20               | 80                                | 191   | 282                     | 228   | do       | Soft.                                   |

## Preparation

This composition was prepared the same as in Example I except that no sodium soap was prepared.

## EXAMPLE III

## Formulation

| Ingredients:                                | Weight per cent |
|---------------------------------------------|-----------------|
| Hydrogenated fish oil acids                 | 20.00           |
| Magnesium hydroxide                         | 4.15            |
| Sodium hydroxide                            | 1.42            |
| Mineral lubricating oil (70 SUS at 210° F.) | 74.43           |

## Preparation

This composition was prepared as in Example I except that no lithium soap was formed.

## EXAMPLE IV

## Formulation

| Ingredients:                                | Weight per cent |
|---------------------------------------------|-----------------|
| Hydrogenated fish oil acids                 | 20.00           |
| Magnesium hydroxide                         | 8.30            |
| Mineral lubricating oil (70 SUS at 210° F.) | 71.70           |

## Preparation

This composition was prepared as in Example I except that no lithium or sodium soap was prepared.

## EXAMPLE V

## Formulation

| Ingredients:                                | Weight per cent |
|---------------------------------------------|-----------------|
| Hydrogenated fish oil acids                 | 10.00           |
| Lithium hydroxide                           | 1.40            |
| Mineral lubricating oil (70 SUS at 210° F.) | 88.60           |

## Preparation

This composition was prepared as in Example I except that no magnesium or sodium soap was formed.

## EXAMPLE VI

## Formulation

| Ingredients:                                | Weight per cent |
|---------------------------------------------|-----------------|
| Hydrogenated fish oil acids                 | 14.00           |
| Sodium hydroxide                            | 2.00            |
| Mineral lubricating oil (70 SUS at 210° F.) | 84.00           |

These results are also shown pictorially in the accompanying drawing. In the drawing the micro-penetration of the samples are plotted against the number of hours subjected to the test temperature. It is graphically shown in the drawing that whereas the composition of invention remained uniformly stable for the duration of the test, the greases of the comparative examples softened to a great extent with subjection to the test temperature.

The lubricating grease compositions of this invention have been found to be compatible with various of the well known additive materials which may be included. There may be blended with these compositions such materials as antioxidants, tackiness agents, color improvers and the like without detracting from the desirable characteristics of the compositions.

To summarize briefly this invention relates to improved magnesium greases which consist essentially of a lubricating oil base stock thickened to a grease consistency with a combination of the magnesium, lithium and sodium soaps of fatty acids. The total amount of soap will be dependent upon the consistency desired in the final product but will preferably vary from about 10.0% to about 25.0% by weight based on the weight of the total composition. The proportion of the component parts of the total mixture may vary from about 0.5 to 5 mols of lithium and sodium soap per mole of magnesium. The preferred embodiment, however, contemplates the use of one mol of lithium soap and one mol of sodium soap for two mols of magnesium soap to thicken to a grease consistency a mineral oil distillate having a viscosity from 35 to 1000 SUS at 100° F. The greases are prepared by forming first the magnesium soap, then the lithium soap, and finally the sodium soap in a mineral oil, heating to about 300° F. and then cooled without stirring.

What is claimed is:

1. A lubricating grease composition which consists essentially of a lubricating oil base stock containing combined therein a grease forming amount of a mixture of magnesium, lithium, and sodium soaps of high molecular weight fatty acids, said mixture containing a molar ratio of magnesium to lithium to sodium soaps of from 5:1:1 to 1:5:5.

2. A composition according to claim 1 wherein there is present from 5.0 to 30.0% by weight of the total soap mixture.

3. A composition according to claim 1 wherein the lu-

bricating oil has a viscosity at 210° F. within a range of from 35 to 1000 SUS.

4. A lubricating grease composition consisting essentially of a mineral lubricating oil base stock thickened to a grease consistency with from about 10.0% to 25.0% by weight of a mixture of soaps comprising about 2 molar proportions of a magnesium soap with about 1 molar proportion of lithium soap and about 1 molar proportion of sodium soap.

5. A process for the preparation of lubricating greases which comprises the steps of forming a magnesium soap in a mineral lubricating oil, then forming a lithium soap and a sodium soap respectively, heating the total mixture

to above the transition point of the soaps, adding additional mineral oil, and then cooling the heated mixture.

References Cited in the file of this patent

UNITED STATES PATENTS

|           |          |       |               |
|-----------|----------|-------|---------------|
| 2,293,052 | Earle    | ----- | Aug. 18, 1942 |
| 2,397,956 | Fraser   | ----- | Apr. 9, 1946  |
| 2,409,950 | Meyer    | ----- | Oct. 22, 1946 |
| 2,417,429 | McLennan | ----- | Mar. 18, 1947 |
| 2,417,431 | McLennan | ----- | Mar. 18, 1947 |

FOREIGN PATENTS

|       |               |       |              |
|-------|---------------|-------|--------------|
| 1,659 | Great Britain | ----- | Mar. 1, 1890 |
|-------|---------------|-------|--------------|